

## UNITED STATES PATENT OFFICE

2,196,101

## LUBRICATING OIL

Emmett C. Carmichael, Jackson Heights, Richard J. De Gray, Forest Hills, and John H. Prall, Brooklyn, N. Y., assignors to Socony-Vacuum Oil Company, Incorporated, New York, N. Y., a corporation of New York

No Drawing. Application September 23, 1938,  
Serial No. 231,328

11 Claims. (Cl. 87—9)

This invention relates to improved lubricating oils.

In one aspect it relates to improved oils used in rolling mill operations, particularly in rolling alloy steels and aluminum.

In another aspect it relates to improved lubricating oils for lubrication of steam cylinders, air compressors, vacuum pumps, and for similar service.

10 It is one of the objects of this invention to provide roll oils of increased film strength which in turn raises the efficiency of rolling operation by allowing the application of higher pressures to the rolls and obtaining a higher reduction of metal per pass. A further object is to provide roll oils capable of preferential wetting of metals in the presence of water. It is also the object of this invention to provide roll oils which are non-corrosive to metals under the processing conditions existing at the rolling mills during the rolling and annealing steps, and which lead to the production of stain-free, bright metal surfaces upon annealing and conventional burnishing. Particularly, the present invention is intended to 15 solve difficulties associated with the rolling and annealing of alloy steels such as stainless steel, and of aluminum.

While heretofore some of the above objectives were partly attained by mineral and fatty oils, or 20 by mixtures thereof, the present invention enables the trade to attain them simultaneously.

It is another of the objects of this invention to provide lubricants which possess greatly decreased tendency to carbonize in service in steam 25 and gas engines and air compressors, which in turn leads to increased efficiency in operation and prolonged cycles between the shut downs for cleaning purposes. It is also the object of this invention to provide lubricants with highly pronounced preferential wetting power toward metals, or in other words, with higher resistivity to the washing effect of steam, air, gas and condensate. The novel oils also lend themselves readily to atomization.

45 Roll oils are used in metal rolling mills in the process of conversion of the billets into sheets and strips and also for further reduction of the sheets and strips to specified gauge. The roll oil is applied to the metal just before it passes between the rolls where the reduction to gauge takes place. Several passes through roll stands are usually required, and each pass involves the application of roll oil. The latter may be used straight or concurrently with a water spray. The function 50 of the roll oil is lubrication, prevention of oxidation of the metal and removal of heat. In order to perform these functions satisfactorily, the roll oil must be non-corrosive, possess adequate wetting power toward dry or water wet metals, and 55 form a film of sufficient strength to withstand the

pressure of the rolls. Furthermore, subsequent to the rolling, the manufactured metal goods may be subjected to an annealing process to relieve the stresses in the metal. The annealing comprises heating, in either reducing or oxidizing atmosphere, to a high temperature specific to the particular metal under treatment, followed by comparatively slow cooling. As the temperatures prevailing in the annealing ovens are in the range of 550° F. to 2000° F., the roll oil film partly volatilizes and partly decomposes. It is essential that no stains or oxide films not removable by conventional burnishing operations remain on the metal as a result of incomplete removal, or carbonization of the roll oil, or of any chemical reaction between the roll oil and the metal. Otherwise, the removal of unsightly oxide films and stains would involve prohibitive mechanical cleaning or rejection.

20 A wide variety of oils, such as mineral hydrocarbon oils, made from petroleum by known methods of refining; fatty oils of animal and vegetable origin, as well as blends of mineral and fatty oils, with and without emulsifiers, have been used for metal rolling.

25 We have discovered that a roll oil consisting of a high percentage of mineral oil and a small percentage of nitrated fatty oil possesses outstanding performance characteristics not observed in similar products known to the art heretofore.

30 As an example of improved roll oil covered by this invention, we may cite the following composition:

|                             | Per cent |
|-----------------------------|----------|
| Nitrated tallow             | 2        |
| Paraffin oil                | 98       |
| Gravity, °A. P. I.          | 31.1°    |
| Flash, C. O. C., °F.        | 315      |
| S. U. viscosity @ 100° F.   | 54"      |
| Color                       | Light 4½ |
| Conradson carbon residue, % | 0.09     |
| Pour, °F.                   | 5        |

40 The physical properties of the blend are as follows:

|                             |          |
|-----------------------------|----------|
| Gravity, °A. P. I.          | 31.1°    |
| Flash, C. O. C., °F.        | 315      |
| S. U. viscosity @ 100° F.   | 54"      |
| Color                       | Light 4½ |
| Conradson carbon residue, % | 0.09     |
| Pour, °F.                   | 5        |

45 Mineral oils, such as made by refining of petroleum have been known as satisfactory lubricants for a wide variety of applications. However, there are numerous cases in which the oil film has to withstand the action of air, gas, steam and condensate at high pressures and temperatures. In steam, compressor and vacuum pump cylinder lubrication, e. g., there is a sweeping effect of the flowing steam and air respectively, at high temperatures, pressures, and velocities of flow. In 50 addition to this mechanical action, condensed water which is present in saturated steam and in compressed air at high pressures, tends to replace the oil film on the metal surfaces. The difficulties of lubrication are augmented by carbon deposits 55

60

in various parts of the engines, particularly on the exhaust valves and in piston grooves because of the decomposition of hydrocarbons under the described severe operating conditions.

5 For better distribution of the lubricant inside the cylinder and for lower consumption, it has been found advantageous, in certain cases, to introduce the lubricant in a finely atomized state. This method has been widely used in steam cylinder lubrication.

10 In order to meet the above requirements in cases in which straight hydrocarbon oils have failed, so-called compounded lubricants have been developed and used. The latter consist of 15 mineral oils of proper characteristics and comparatively small admixtures of fatty oils and fatty acids of animal and vegetable origin. Tallow, neat's-foot oil, and elaine oil are common examples of fatty materials in compounded lubricants 20 of the above classes. Compounded oils have shown better performance than straight mineral oils with respect to metal wetting, ease of atomization and softer carbon deposits.

25 We have discovered that compounded lubricants consisting of hydrocarbon oils of appropriate viscosity and other characteristics, and of smaller amounts of nitrated fatty oil possess outstanding properties for meeting the conditions existing in steam engine, gas engine, vacuum 30 pump, and air compressor lubrication, and in similar service.

35 The following composition formulae are representative of the novel cylinder lubricants disclosed in the present specification:

|                                 |                               | Compressor oil | Cylinder oil |
|---------------------------------|-------------------------------|----------------|--------------|
| 40                              | Nitrated tallow.....percent.. | 0.75           | 4.00         |
|                                 | Mineral oil.....do.....       | 99.25          | 96.00        |
| <i>Physical characteristics</i> |                               |                |              |
| 45                              | Gravity.....°A. P. I.         | 26.0           | 24.6         |
|                                 | Flash, open cup.....°F.       | 400            | 585          |
|                                 | Saybolt Universal viscosity:  |                |              |
|                                 | @ 100° F.                     | 314"           | 4200"        |
|                                 | @ 210° F.                     |                | 220"         |
|                                 | Color, A. S. T. M.....        | Dark 1½        | Dark green   |

50 The nitrated tallow is a product of reaction between common tallow and concentrated nitric acid. When the two reactants are heated to 220-230° F., an exothermal reaction occurs, the temperature rising to 250-280° F. without additional heat. The excess mineral acid is washed out with water, upon cooling, and the product is dried. The following table illustrates the properties of the original common tallow and the nitrated tallow:

|    | Common tallow          | Nitrated tallow |
|----|------------------------|-----------------|
| 60 |                        |                 |
|    | Acid number.....       | 9.7             |
|    | Ester No.....          | 106.1           |
|    | Saponification No..... | 206.8           |
|    | Iodine No.....         | 53.8            |
|    | Titer, °C.....         | 35.4            |
| 65 |                        | 26.0            |
|    | 104.3                  |                 |
|    | 220.3                  |                 |
|    | 30.0                   |                 |
|    | 31.0                   |                 |

70 The paraffin oil (used in roll oils) is a light mineral oil of approx. 50 seconds viscosity at 100° F. (Saybolt Universal).

75 The blended roll oil is prepared by simple stirring of the two ingredients at a temperature above the melting point of the nitrated fat.

The mineral oils used in the above cylinder oil formulae are hydrocarbon oils made from petroleum by known methods of refining. Their 75 viscosities are 300 vis. Say. Univ. at 100° F. and

230 sec. Say. Univ. at 210° F. for the compressor oil and the steam cylinder oil, respectively.

The nitrated tallow and mineral oil are combined by mixing at a temperature above the melting point of the nitrated fat.

Subject to various applications in compressor, vacuum pump, gas engine and steam cylinder lubrication, the mineral oils may vary in broad limits. E. g., the preferred ranges for steam cylinder and compressor oils are as follows:

|                              | Minimum               | Maximum               |
|------------------------------|-----------------------|-----------------------|
| For steam cylinder oils..... | 60" S. U. vis. @210.  | 300" S. U. vis. @210. |
| Compressor oils.....         | 150" S. U. vis. @100. | 600" S. U. vis. @100. |

10

15

The nitrated tallow is representative of a broad group of animal and vegetable fatty oils, such as sperm oil, palm oil, lard oil, and the like, containing unsaturated components and susceptible to nitration. The degree of nitration can be varied and is not limited to the above example. The decrease in iodine number of the fatty oil is a convenient measure of the degree of nitration. While in the above example, the nitrated tallow shows an iodine number 23.8 points lower than the original tallow, (30 vs. 53.8), more or fewer nitro groups can be introduced, the upper limiting point being the stability of the solution of the nitrated product in mineral oil. E. g., common tallow can be nitrated to final iodine numbers ranging from 50 to 15. For other fatty oils these numerical values are different.

25 The percentage of the nitrated fatty oil in the finished lubricant may be changed within the following limits: 0.25% to 25%.

30 The composition of the novel lubricants covered by this invention is not limited to a binary blend of mineral oil and nitrated fat. It has been found advantageous, in certain cases, to add nitrated fat, within the above limits, to compounded oils already containing fats or fatty acids. As an example of such product, we may cite the following formula of a steam cylinder oil:

|                                               | Per cent |
|-----------------------------------------------|----------|
| Mineral oil 150 sec. Say. Univ. @ 210° F..... | 92       |
| Acidless tallow.....                          | 7        |
| Nitrated tallow.....                          | 1        |

45

50

55 The relative load carrying capacities of roll oils can be conveniently indicated by the Almen pin test described by Moughay and Almen (Proc. A. P. I., 1931, page 77). This test is conducted in a specially designed machine the essential parts of which are a rotating pin and a bearing lubricated with the oil in question. Increasing loads are applied to the lubricated surface until the oil film fails. The following tabulation shows the effect of addition of nitrated fat to a 100" paraffin oil.

| Product                                         | Lbs./sq. in. load before failure |
|-------------------------------------------------|----------------------------------|
| 100" Saybt. Univ. @ 100° F. paraffin oil.....   | 3000                             |
| Same+2% nitrated sperm oil.....                 | 5500                             |
| Same+2% nitrated tallow.....                    | 6000                             |
| Same+3% nitrated sperm oil.....                 | 6500                             |
| Same+3% nitrated tallow.....                    | 7000                             |
| Same+5% nitrated sperm oil.....                 | 9000                             |
| Same+9% nitrated sperm oil.....                 | 13000                            |
| Commercial roll oil (containing 7% degras)..... | 3000                             |

60

65

70

75 It will be noted that the nitrated fat definitely imparts film strength while the addition of original fatty materials has no effect on the load carrying capacity of the mineral oil.

75

The ability of the novel roll oils to leave a bright metal surface after exposure to high temperature in annealing ovens can be demonstrated by the following comparative tests:

5 Highly polished plates of 18-8 chromium nickel stainless steel were slushed with various roll oils and annealed at 1700° F. for 3 minutes in an oxidizing atmosphere. The inspection of the plates disclosed the following results:

| 10 | Product                                                             | Appearance of metal surface       |
|----|---------------------------------------------------------------------|-----------------------------------|
| 1  | Paraffin oil 50 sec. S. U. vis. @ 100° F.                           | Dull oxide coating, no rust.      |
| 2  | Same 98%+2% nitrated tallow                                         | Bright clean oxide film; no rust. |
| 15 | 3 Same 98%+2% nitrated sperm oil                                    | Do.                               |
| 4  | 4 Same 90%+10% niger palm oil                                       | Rust spots.                       |
| 5  | 5 Niger palm oil                                                    | Do.                               |
| 20 | 6 Commercial roll:<br>93% 50 sec. @100° F. paraffin oil 7% degrads. | Rust stains.                      |

The best way of proving the value of the lubricating oils covered by this invention is field testing in full size engines. This has been done on steam and gas engines, compressors and vacuum pumps and reports are on hand confirming the fine performance, particularly the low carbonization tendency and high preferential wetting power of the oils containing the nitrated fats.

25 We claim:

- 30 1. Improved mineral lubricant oil compositions comprising a major proportion of a viscous mineral lubricating oil fraction and a minor proportion of a nitrated fatty oil.
2. A mineral lubricant oil composition comprising a viscous mineral lubricating oil fraction and in addition thereto a small proportion, from about 0.25% to about 25.0% of a nitrated fatty oil.
- 35 3. A mineral lubricating oil composition com-

prising a viscous mineral oil fraction and in addition thereto a small proportion of nitrated tallow.

4. A mineral lubricating oil composition comprising a viscous mineral oil fraction and in addition thereto a small proportion of tallow nitrated to an iodine number of from 50 to 15.

5. A mineral lubricating oil composition comprising a viscous mineral oil fraction and in addition thereto from 0.25% to 25.0% of tallow nitrated to an iodine number of from 50 to 15.

10 6. A lubricant composition for use in rolling operations comprising a light viscous mineral oil fraction and from 0.25% to 25.0% of nitrated tallow.

15 7. A lubricant composition for use in rolling operations comprising a light viscous mineral oil fraction and about 2% of nitrated tallow.

8. A lubricant composition for use in rolling operations comprising a light viscous mineral oil fraction of about 2% of nitrated tallow having an iodine number of about 30.

20 9. A lubricant composition for use in lubrication of steam cylinders, compressors, and the like, comprising a heavy viscous mineral oil fraction and from 0.25% to 25.0% of nitrated tallow.

25 10. A lubricant composition for use in steam cylinders, compressors, and the like comprising a heavy viscous mineral oil fraction and from about 0.75% to about 4.0% of nitrated tallow.

30 11. A lubricant composition for use in steam cylinders, compressors, and the like comprising a heavy viscous mineral oil fraction and from about 0.75% to about 4.0% of nitrated tallow having an iodine number of about 30.

EMMETT S. CARMICHAEL.  
RICHARD J. DE GRAY.  
JOHN H. PRALL.